

**United States Patent [19]**

Taylor

[ 19 ]

[11] 3,770,439

[45] Nov. 6, 1973

- [54] **POLYMERIC MORDANT IN COLOR DIFFUSION TRANSFER IMAGE RECEIVING LAYER**

[75] Inventor: **Lloyd D. Taylor, Lexington, Mass.**

[73] Assignee: **Polaroid Corporation, Cambridge, Mass.**

[22] Filed: **Jan. 3, 1972**

[21] Appl. No.: **215,082**

- [52] U.S. Cl. .... 96/77, 96/3, 96/290  
[51] Int. Cl. .... G03c 1/40  
[58] Field of Search ..... 96/29 D, 3, 77

[56] References Cited

UNITED STATES PATENTS

- |           |         |            |         |
|-----------|---------|------------|---------|
| 3,239,337 | 3/1966  | Haas ..... | 96/29 D |
| 3,249,432 | 5/1966  | Haas ..... | 96/77   |
| 3,415,644 | 12/1968 | Land ..... | 96/29 D |

*Primary Examiner*—Norman G. Torchin  
*Assistant Examiner*—Richard L. Schilling  
*Attorney*—Brown & Mikulka

[57]

## ABSTRACT

A photographic product having an image pattern receiving layer which comprises a polymer of the formula:



### Formula A

where each R<sup>1</sup> can be the same or different substituent chosen from the group consisting of hydrogen, alkyl, alkoxy and alkanol and X<sup>-</sup> is an anion radical.

**13 Claims, No Drawings**

## POLYMERIC MORDANT IN COLOR DIFFUSION TRANSFER IMAGE RECEIVING LAYER

### BACKGROUND OF THE INVENTION

#### 1. The Field of the Invention

This invention relates to photographic products. More precisely, the invention disclosed herein relates to photographic products especially useful in providing image patterns by way of diffusion transfer photographic processes.

#### 2. Description of the Prior Art

Diffusion transfer photographic processes and photographic products adapted for such processes are well known to the art. Essentially, such products and processes involve a photosensitive system which is exposed to an image pattern of activating radiation. After exposure, the resultant image pattern can be developed to provide a diffusion transfer image pattern which can be transferred to an image pattern receiving layer. Details relating to some of the better known diffusion transfer photographic products and processes can be found in U. S. Pat. Nos. 2,983,603; 3,415,644; 3,415,645; 3,415,646; 3,473,925; 3,573,042; 3,573,043; 3,573,044; 3,576,625; 3,576,626; 3,578,540; 3,579,333; 3,473,925; 3,594,164 and 3,594,165 as well as in commonly assigned U. S. Pat. application Ser. Nos. 782,056, now U.S. Pat. No. 3,672,486; 782,075, now abandoned, both filed Dec. 9, 1969 and U. S. Pat. application Ser. No. 65,084 filed Aug. 19, 1970, now U.S. Pat. No. 3,672,890. All of the above patents and applications are expressly incorporated herein in their entirety by reference.

Photosensitive systems employed in the products and processes of the type described in the above-mentioned patents and applications comprise at least one selectively sensitized silver halide layer integrated with a dye image-providing material. More often, however, such diffusion transfer photographic products and processes include a photosensitive system which can provide multicolor diffusion transfer image patterns and photosensitive systems of this type essentially include a blue, a green and a red sensitive silver halide layer each integrated respectively with a yellow, a magenta and a cyan dye image-providing material.

Suitable dye image-providing employed in diffusion transfer photosensitive systems are those which are either (1) initially soluble or diffusible in the processing composition but are selectively rendered non-diffusible as a function of development; or (2) initially soluble or non-diffusible in the processing composition but are selectively rendered diffusible as a function of development. Accordingly suitable dye image-providing materials may be complete dyes or dye intermediates, e.g., color couplers and especially preferred materials are those known to the art as "dye developers," e.g., a dye which is also a silver halide developing agent.

Examples of and details relating to initially soluble or diffusible materials and their application in color diffusion transfer, can be found in U. S. Pat. Nos. 2,647,049; 2,661,293; 2,698,244; 2,698,798; 2,802,735; 2,774,668 and 2,983,606. Examples of and details relating to diffusion transfer systems employing initially non-diffusible materials can be found in U. S. Pat. Nos. 3,443,939; 3,443,940; 3,227,550; 3,227,551; 3,227,552; 3,227,554; 3,243,294; and 3,445,228.

A known diffusion transfer particularly suitable for providing monochrome or multicolor image patterns of

or comprising green, cyan and blue colors is one employing phthalocyanine dye developers of the type described in U. S. Pat. No. 3,482,972 issued to Elbert M. Idelson on Dec. 9, 1969. Dye developers of the type disclosed there are those conforming to the following formula:



FORMULA B

where that of the 16 R substituents present on the phthalocyanine ring at least one and no more than four are as R¹ groups, there being no more than two R¹ groups on any one benzene ring, the remaining R substituents being R² groups, and R¹ comprises a group  $(-A)_n-E$ ; A is a divalent organic linking radical; n is a number of from 0-1; E is an aryl group selected from the group consisting of benzene and naphthalene radicals so substituted by at least two groups selected from the group consisting of hydroxyl and amino groups which are situated ortho or para to each other as to be capable of developing an exposed silver halide photographic emulsion; M is a metal selected from the group consisting of cobalt, nickel, copper, chromium, magnesium and zinc; and each R² comprises the same or a different moiety selected from the group consisting of monovalent organic and monovalent inorganic radicals, neither of which contain a silver halide developing radical, and hydrogen. Most preferred are those cyan dyes within the above formula wherein the metal moiety is copper and these dye developers may be referred to simply as copper phthalocyanine dye developers.

### SUMMARY OF THE INVENTION

The present invention provides novel image receiving layers and diffusion transfer photographic products employing such layers. Essentially the image receiving layers of the present invention are water permeable, substantially water insoluble, dimensionally stable layers comprising a polymeric material including a polymer of the formula:



Formula A.

where each R<sup>1</sup> can be the same or different substituent chosen from the group consisting of hydrogen, hydroxyl, alkyl, alkoxy or alkanol and preferably lower alkyl, alkoxy or alkanol, e.g., wherein the hydrocarbon moiety contains one to six carbon atoms and X<sup>-</sup> is an anion radical.

Representative polymers of Formula A include those conforming to the following specific structural formulae:

(1)



(2)



(3)



(4)



(5)



Polymeric materials conforming to the above formula have been found to be especially effective as mordants

for dye image providing materials and especially effective as mordants for the phthalocyanine dye developers mentioned before. Accordingly, photographic products containing the novel image receiving layers are particularly suitable for providing high quality, colored, diffusion transfer image patterns consisting of or comprising cyan, green or blue colors provided by phthalocyanine dye developers.

10

#### DESCRIPTION OF THE PREFERRED EMBODIMENTS

As mentioned, the image receiving layers of the present invention essentially comprise a polymer of Formula A. More precisely, however, the image receiving layers of the present invention comprise a polymer of Formula A copolymerized with other polymeric materials or preferably a physical blend of other polymeric materials and a polymer of Formula A. Other polymeric materials which can be included in the copolymers or in the mixtures or blends comprising the image receiving layers of the present invention are those compatible polymeric materials which can provide substantially transparent water permeable and/or swellable but substantially water insoluble, dimensionally stable layers. Specific suitable polymeric materials that can be included in the image receiving layers copolymerized with or most preferably in physical admixture with a polymeric material of Formula A include the polymers and copolymers of polyvinyl alcohol, polyacrylamide, polyvinyl pyridine and polyhydroxyalkylcellulose such as polyhydroxymethylcellulose, polyhydroxyethylcellulose, etc. Especially suitable receiving layers include a mixture or blend of polyacrylamide, and/or polyhydroxyalkylcellulose together with poly-4-vinylpyridine and a polymeric material of Formula A where the concentration of the polymeric material of Formula A ranges from about 8 percent by weight of the total weight of polymeric materials in the blend to about 50 percent by weight or somewhat higher. Polymeric materials of Formula A as well as those that can be mixed or blended therewith to provide image receiving layers of the present invention are commercially available. The particular additional polymeric materials selected to be employed in the mixture and the respective amounts of each will be determined primarily by the balance of properties and characteristics desired of the layer, e.g., the strength, the swellability or moisture permeability of the layer. The molecular weight of the polymeric materials employed in the mixtures or blends is not an especially critical feature and is subject to normal considerations such as the case of dispersion of the material in a selected dispersion medium or the compatibility of the polymeric material with other ingredients of the mixture and/or with the dispersion medium.

#### DESCRIPTION OF THE PREFERRED EMBODIMENT

The following illustrates some of the advantages and benefits to be obtained in accordance with the practice of the present invention. In order to illustrate these advantages and benefits by way of comparative data, diffusion transfer photographic products were prepared which comprised the following layers and/or elements:

1. a layer of cyan dye developer dispersed in gelatin and coated at a coverage of about 100 mgs./ft.<sup>2</sup> of dye and about 150 mgs./ft.<sup>2</sup> of gelatin;

2. a red-sensitive gelatino silver iodobromide emulsion coated at a coverage of about 140 mgs./ft.<sup>2</sup> of silver and about 50 mgs./ft.<sup>2</sup> of gelatin;

3. A layer of a 60-30-4-6 copolymer of butylacrylate, diacetone acrylamide, styrene and methacrylic acid and polyacrylamide coated at a coverage of about 150 mgs./ft.<sup>2</sup> of the copolymer and about 5 mgs./ft.<sup>2</sup> of polyacrylamide;

4. a layer of magenta dye developer dispersed in gelatin and coated at a coverage of about 100 mgs./ft.<sup>2</sup> of dye and about 150 mgs./ft.<sup>2</sup> of gelatin;

5. a green-sensitive gelatino silver iodobromide emulsion coated at a coverage of about 120 mgs./ft.<sup>2</sup> of silver and about 35 mgs./ft.<sup>2</sup> of gelatin;

6. a layer containing the copolymer referred to above in layer 3 and polyacrylamide coated at a coverage of about 100 mgs./ft.<sup>2</sup> of copolymer and about 12 mgs./ft.<sup>2</sup> of polyacrylamide;

7. a layer of yellow dye developer dispersed in gelatin and coated at a coverage of about 70 mgs./ft.<sup>2</sup> of dye and about 105 mgs./ft.<sup>2</sup> of gelatin;

8. a blue-sensitive gelatino silver iodobromide emulsion layer including the auxiliary developer 4'-methylphenyl hydroquinone coated at a coverage of about 80 mgs./ft.<sup>2</sup> of silver, about 25 mgs./ft.<sup>2</sup> of gelatin and about 15 mgs./ft.<sup>2</sup> of auxiliary developer; and

9. a layer of gelatin coated at a coverage of about 50 mgs./ft.<sup>2</sup> of gelatin.

The three developers employed above were the following:



a cyan dye developer;



6  
a magenta dye developer; and



a yellow dye developer.

Then a transparent 4 mil. polyethylene terephthalate film base was coated, in succession, with the following illustrative layers:

1. a polymeric acid neutralizing layer containing a 7:3 mixture, by weight, of polyethylene/maleic anhydride copolymer and 88-90 percent hydrolyzed polyvinyl acetate at a coverage of about 1,000 mgs./ft.<sup>2</sup>;

2. a graft copolymer of acrylamide and diacetone acrylamide on a polyvinyl alcohol backbone in a molar ratio of 1:3.2:1 at a coverage of about 800 mgs./ft.<sup>2</sup>, to provide a polymeric spacer or timing layer; and

3. a receiving layer was provided at a coverage of about 300 mgm./ft.<sup>2</sup> comprising a mixture of polyacrylamide, poly-4-vinyl pyridine and an approximately equivalent mixture of polymers of Formula A of the following specific structures:



40 Meta and para Polyvinylbenzyl trimethyl ammonium chlorides

The ratio of each polymeric material to each other was varied in the manner set forth in the example which follows. In the "control" for the example, a mixture of polyacrylamide and poly-4-vinyl pyridine was employed to provide the image receiving layer.

The two components will then be laminated together to provide an integral film unit.

50 A rupturable container comprising an outer layer of lead foil and an inner liner or layer of polyvinyl chloride retaining an aqueous alkaline processing solution was fixedly mounted on the leading edge of each of the laminates, by pressure-sensitive tapes, interconnecting the respective container and laminates so that, upon application of compressive pressure to the container to rupture the container's marginal seal, its contents may be distributed between the image receiving layer and the gelatin layer, (layer 9), of the negative component.

55 60 The processing composition employed in the rupturable container comprised the following properties of ingredients:

Water — 100 cc.

Potassium hydroxide — 11.2 gms.

Hydroxyethyl cellulose high viscosity) [commercially available from Hercules Powder Co., Wil., Del., under the trade name Natrasol 250] — 3.4 gms.

N-phenethyl- $\alpha$ -picolinium bromide — 2.7 gms.  
 Benzotriazole — 1.15 gms.  
 Titanium dioxide — 50.0 gms.

(A)



2.08 gms.

(B)



0.52 gms.

(C)



11.8 gms.

Film units of the foregoing description can be exposed in known manner to form a developable image and the exposed element can then be developed by applying compressive pressure to the rupturable container in order to distribute the aqueous alkaline process composition, thereby forming a multicolor transfer image which is viewable through the transparent polyethylene terephthalate film base as a positive reflection print. As was discussed before, this development may be effected in the presence of actinic light because the negative component is suitably protected from fogging.

#### EXAMPLE

Diffusion transfer film units were prepared in the manner described above. The image receiving layers of each of these film units comprised varying mixtures of polyacrylamide, poly-4-vinylpyridine and the aforementioned approximately 1:1 mixture of the polymers

of Formula A, e.g., poly quaternarys of the following specific structure:



Meta and para Polyvinylbenzyl trimethyl ammonium chlorides sold by Dow Chemical Company under the trade name "E.C.R. 34"

The respective ratios of the ingredients of each mixture employed in the film units are set forth in tabular form below which also describes the composition of the mixture employed to provide an image receiving layer for a "control" film unit.

TABLE I

| 20                    | Film unit no. | Ratio of poly-<br>acrylamide-poly-<br>4-vinyl<br>pyridine poly | Percent by weight of<br>each material in<br>total weight of poly-<br>meric material in<br>mixture |                              |                           |
|-----------------------|---------------|----------------------------------------------------------------|---------------------------------------------------------------------------------------------------|------------------------------|---------------------------|
|                       |               |                                                                | Poly-<br>acryl-<br>amide                                                                          | Poly-<br>4-vinyl<br>pyridine | Polymers<br>of<br>formula |
| P 2241-A              |               | 4/3/2                                                          | 44                                                                                                | 33                           | 23                        |
| P 2241-B              |               | 4/4/1                                                          | 44                                                                                                | 44                           | 12                        |
| P 2241-C              |               | 4/2/2                                                          | 50                                                                                                | 25                           | 25                        |
| P 2241-D              |               | 4/4/4                                                          | 33                                                                                                | 33                           | 33                        |
| P 2241-E              |               | 4/2/6                                                          | 33                                                                                                | 17                           |                           |
| P 2241-G <sup>1</sup> |               | 4/3/0                                                          | 57                                                                                                | 43                           |                           |

30<sup>1</sup> Control.

Diffusion transfer film units of the type described above were exposed and processed at various temperatures. Examination of the resulting image patterns showed the following differential maximum densities which comprise the difference between the maximum and minimum densities recorded for the various colors of the film with a Quantalog Mac Beth Densitometer.

TABLE II

(Processing Temperature 40°F)

| 40                    | Film unit no. | D-MAX |       |      |
|-----------------------|---------------|-------|-------|------|
|                       |               | Red   | Green | Blue |
| P 2241-A              |               | 1.93  | 1.49  | 1.86 |
| P 2241-B              |               | 1.63  | 1.35  | 1.80 |
| P 2241-C              |               | 2.05  | 1.57  | 1.90 |
| P 2241-D              |               | 1.88  | 1.51  | 1.85 |
| P 2241-E              |               | 2.16  | 1.64  | 1.90 |
| P 2241-G<br>(Control) |               | 1.52  | 1.36  | 1.75 |

TABLE III

(Processing Temperature 74°F)

| 55                    | Film unit no. | D-MAX |       |      |
|-----------------------|---------------|-------|-------|------|
|                       |               | Red   | Green | Blue |
| P 2241-A              |               | 2.29  | 1.93  | 2.07 |
| P 2241-B              |               | 2.07  | 1.87  | 2.0  |
| P 2241-C              |               | 2.27  | 1.96  | 2.09 |
| P 2241-D              |               | 2.17  | 1.89  | 2.03 |
| P 2241-E              |               | 2.29  | 1.89  | 2.03 |
| P 2241-G<br>(Control) |               | 1.79  | 1.72  | 1.94 |

TABLE IV

(Processing Temperature 102°F)

| 60                    | Film unit no. | D-MAX |       |      |
|-----------------------|---------------|-------|-------|------|
|                       |               | Red   | Green | Blue |
| P 2241-A              |               | 2.26  | 1.81  | 2.04 |
| P 2241-B              |               | 2.13  | 1.79  | 2.05 |
| P 2241-C              |               | 2.16  | 1.73  | 1.96 |
| P 2241-D              |               | 2.15  | 1.67  | 1.99 |
| P 2241-E              |               | 2.23  | 1.65  | 1.89 |
| P 2241-G<br>(Control) |               | 1.83  | 1.62  | 1.93 |

A comparison of the above data evidences the advantages in improved color reproduction to be obtained by including a polymeric material of Formula A in mixtures of polymeric materials which can provide image receiving layers for diffusion transfer photographic products.

It will be appreciated that the foregoing description is illustrative and the various elements of diffusion transfer film units may be arranged differently and/or may contain additional reagents providing specific, desired functions. The alternative arrangements of these elements and/or selection the selection of additional reagents will be readily apparent to those skilled in the art and per se comprise no part of this invention.

Since certain changes may be made in the above product without departing from the scope of the invention herein involved, it is intended that all matter contained in the above description shall be interpreted as illustrative and not in a limiting sense.

What is claimed:

1. A receiving element for use in photographic diffusion transfer processes comprising a composite structure which comprises a support and an alkali permeable and dyeable polymeric layer comprising a polymer conforming to formula A below:



where each R<sup>1</sup> can be the same or different substituent chosen from the group consisting of hydrogen, hydroxyl, alkyl radicals having from one to six carbon atoms, alkoxy radicals having one to six carbon atoms or alkanol radicals having one to six carbon atoms; and X<sup>-</sup> is an anion radical.

2. A receiving element of claim 1 wherein said polymeric layer comprises a mixture of a polymer of Formula A and a polymeric material chosen from the group consisting of the polymers of polyvinylalcohol, polyacrylamide, polyvinyl pyridine, polyhydroxyalkylcellulose and mixtures of these.

3. A receiving element of claim 2 wherein the concentration of the polymer Formula A in said mixture ranges from about 8 percent by weight of the total polymeric materials in the mixture to about 50 percent by weight.

4. A receiving element of claim 3 wherein said polymeric layer comprises a mixture of a polymer of Formula A and a polymeric material chose from the group consisting of the polymers of polyacrylamide, poly-4-vinyl pyridine, polyhydroxyalkylcellulose and mixtures of these.

5. A receiving element of claim 3 wherein said polymeric material of Formula A is a polyvinylbenzyl trimethyl ammonium chloride.

6. A receiving element of claim 3 wherein said polymeric material of Formula A is a polyvinylbenzyl trimethyl ammonium chloride and said mixture of poly-

meric materials includes polyacrylamide and poly-4-vinyl pyridine.

7. A diffusion transfer photographic product having as essential elements thereof a photosensitive system comprising at least one selectively sensitized silver halide layer integrated with a dye image providing material, a processing composition which can provide a diffusion transfer image pattern after exposure of said photosensitive system and an image receiving element arranged to receive said diffusion transfer image pattern, said image receiving element comprising a composite structure which comprises a support and an alkali permeable and dyeable polymeric layer comprising a polymer conforming to Formula A below:



Formula A

25 wherein each R<sup>1</sup> can be the same or different substituent chosen from the group consisting of hydrogen, hydroxyl, alkyl radicals having from one to six carbon atoms, alkoxy radicals having from one to six carbon atoms or alkanol radicals having from one to six carbon atoms; and X<sup>-</sup> is an anion radical.

30 8. A diffusion transfer product of claim 7 wherein said photosensitive system comprises a blue, green and red sensitive silver halide layer each integrated with a yellow, a magenta and cyan dye image providing material.

9. A diffusion transfer product of claim 10 wherein the concentration of said compound of Formula A in said mixture of polymeric materials comprising said dyeable layer ranges from about 8 percent by weight of said polymeric materials to about 50 percent by weight.

40 10. A diffusion transfer product of claim 7 wherein said polymeric layer comprises a mixture of polymer of Formula A and a polymeric material chosen from the group consisting of the polymers of polyvinylalcohol, polyacrylamide, polyvinyl pyridine, polyhydroxyalkylcellulose and mixtures of these.

45 11. A diffusion transfer product of claim 10 wherein said polymeric layer comprises a mixture of a polymer of Formula A and a polymeric material chosen from the group consisting of the polymers of polyacrylamide, poly-4-vinyl pyridine, polyhydroxyalkylcellulose and mixtures of these.

50 12. A diffusion transfer product of claim 10 wherein said polymeric material of Formula A in said dyeable layer is a polyvinylbenzyl trimethyl ammonium chloride.

55 13. A diffusion transfer product of claim 10 wherein said polymeric material of Formula A in said dyeable layer is a polyvinyl trimethyl ammonium chloride and said mixture of polymeric materials includes polyacrylamide and poly-4-vinyl pyridine.

\* \* \* \* \*